# EUROPEAN PATENT SPECIFICATION

(11) **EP 1 679 390 B1**
(45) Date of publication and mention of the grant of the patent: **08.08.2012**
(21) Application number: 05112620.9
(22) Date of filing: 21.12.2005
(51) Int. Cl.: C23C 18/12, F01D 5/28

(54) **Method for forming a protective layer on a metallic turbine substrate**
Verfahren zur Herstellung von Schutzschichten auf einem Substrat einer metallische Turbine
Methode pour former une couche protectrice sur un substrat d'une turbine métallique

(30) Priority: 11.01.2005 IT TO20050008
(43) Date of publication of application: 12.07.2006
(73) Proprietor: AVIO S.p.A., 10135 Torino (IT)
(72) Inventor: Badini, Claudio, 10126 Torino (IT); Fino, Paolo, 10134 Torino (IT); Biamino, Sara, 14100 Asti (IT); Sabbadini, Silvia, 10134 Torino (IT); Zanon, Giovanni, 10040 Rivalta di Torino (IT)
(74) Representative: Jorio, Paolo

(56) References cited:
- EP-A- 1 170 251
- US-A- 5 318 800
- US-A- 5 955 145
- US-A- 6 001 416
- PATENT ABSTRACTS OF JAPAN vol. 017, no. 345 (C-1077), 30 June 1993 (1993-06-30) & JP 05 043839 A (SEKISUI CHEM CO LTD), 23 February 1993 (1993-02-23)
- GADOW R ET AL: "LANTHANUM HEXAALUMINATE - NOVEL THERMAL BARRIER COATINGS FOR GAS TURBINE APPLICATIONS - MATERIALS AND PROCESS DEVELOPMENT" SURFACE AND COATINGS TECHNOLOGY, ELSEVIER, AMSTERDAM, NL, vol. 151/152, 2002, pages 392-399, XP001121228 ISSN: 0257-8972
- FEI LI, KEAO HU, JIANLIN LI, DONG THANG, GANG CHEN: "Combustion synthesis of gamma-lithium aluminate by using various fuels" J. OF NUCLEAR MATERIALS, vol. 300, 2002, pages 82-88, XP002427793
- BYUNG-KWAN IKIM AND I. YASUI: "Synthesis of Fine Particles of hydrated Al2O3 and Al2O3-coated Cr2O3 Composite Powders by the Homogeneous Precipitation Method" J. CER. SOC. , JPN INTERN ED., vol. 95, 1987, pages 399-405, XP008077192
- RAO R R ; MARIAPPAN L: "Combustion synthesis and characterisation of lanthanum hexa-aluminate" ADV. APPL. CERAM.; ADVANCES IN APPLIED CERAMICS, vol. 104, no. 5, October 2005 (2005-10), pages 268-271, XP008077197

## Description

The present invention relates to a method for forming a protective layer with the functions of protecting against oxidation and corrosion and acting as a thermal barrier on a metallic turbine substrate, and also relates to the metallic turbine substrate produced by means of the method.

The turbines used in the aerospace field are subjected to considerable thermal stresses due to the high temperatures of 1400°C and above reached by the combustion products formed in turbine engines. If such temperatures are reached, the metallic components of the turbine, particularly the blades, which generally consist of nickel based superalloys, can be subject to structural deformation and corrosion and oxidation phenomena which may adversely affect their operation.

There is a known way of forming a protective layer on the surfaces of the metallic components, to act as a thermal barrier in order to protect the turbines from the high operating temperatures.

At the present time, the known and widely used processes for forming a protective layer are called "Air Plasma Spraying", also known by the acronym "APS", and referred to in this way in the following text, and "Electronic Beam Physical Vapour Deposition", also known by the acronym "EB-PVD" and referred to in this way in the following text.

In the APS method, a flow of a first inert gas, for example argon, is made to contact the surfaces of electrodes which cause the gas to become ionized. the ionized gas thus produced, also called "plasma", is sprayed into a chamber into which is simultaneously introduced, through an inlet tube, the powder of the material which is to form the protective layer, suspended in a flow of a second inert gas. When the high-temperature plasma comes into contact with the powder, it fuses the latter to form droplets. The droplets produced in this way are sprayed on to the surface to be coated.

This deposition method enables protective layers with very low heat conduction to be obtained, but, owing to the structure of the material forming the protective layer, has a very low resistance to thermal fatigue by comparison with thermal barriers produced by the EB-PVD method; indeed, it tends to crumble if repeatedly subjected to high temperatures.

Moreover, the APS method provides good results only if the protective layer is applied to surfaces with a high degree of roughness.

An example of such APS method is disclosed by Gadow R. et al "Lanthanum hexaaluminate - novel thermal barrier coatings for gas turbine applications - Materials and prozendevelopment" in Surface and Coating Technology 151-152 (2002) 392-399.

In the EB-PVD method, the material which is to constitute the protective layer is in the form of powder placed in a crucible, or is in ingot form. By means of a gun which produces high-energy electron beams, the material is vaporized by the electron beams and then condensed on the surface to be coated.

This method yields protective layers having characteristics which are the opposite of those obtained by the APS method, and indeed these layers have high resistance to both thermal and mechanical stress, but also have high thermal conductivity. A further disadvantage of this deposition method lies in the very high costs of the equipment used.

Finally, both the APS and the EB-PVD method generate protective layers with a coarse structure; in other words, under micrographic examination they are found to have large particle sizes and, owing to the procedure by which the deposition is carried out, they cannot be used to produce protective layers on any microcavities or nonuniformities which may have formed on the metallic substrate.

EP1170251 discloses a process and a composition for forming a metal oxide thin film containing a salt of an amine and a metal complex formed of a ligand having 5 or less coordination and a metal compound is provided.

US 6001416 discloses an oxide thin film comprising an oxide represented by AB03, wherein A comprises at least one element selected from the group consisting of the groups IA, IIA, IIIA, IVB and VB of the periodic table, and B comprises at least one element selected from the group consisting of the groups IVA and VA of the periodic table, wherein said oxide thin film has a mixed structure in which crystal grains are dispersed in an amorphous phase or an ultrafine grain phase.

US 5318800 discloses a method is disclosed of forming thin uniform micron range and submicron range aberration-resistant and hole-free high-temperature thermally stable metal oxide coatings upon metal, insulating and other substrates, involving the application of a polymer metal complex precursor solution to the substrate and appropriate firing for oxidation of the metal and the coating while burning off all traces of the polymer.

In US 5955145 a process for forming a coated article having a wear resistant coating that minimizes the generation and effects of wear debris is provided.

None of the above patent resolves the aforementioned problems.

The object of the present invention is therefore to provide a method for forming a protective layer which resolves the problems described above. In particular, it would be preferable to find a method for depositing a protective layer which resists not only high temperatures but also mechanical stresses, while having low thermal conductivity and being reliable and inexpensive.

According to the present invention, this object is achieved by means of a method for forming a protective layer on a metallic turbine substrate according to Claim 1.

The method according to the present invention can be used to obtain a protective layer which provides thermal protection, consisting of a porous ceramic material based on pure or mixed ceramic oxides. Preferably, the protective layer comprises an oxide selected from the group consisting of ZrO₂, ZrO₂+Y₂O₃, ZrO₂+CaO, Al₂O₃, Al₂O₃+SiO₂, Al₂O₃+TiO₂, CeO₂, BaZrO₃, Y₃Al₅O₁₂, LaMgAl₁₁O₁₉, LaMnAl₁₁O₁₉.

Even more preferably, the protective layer comprises LaMnAl₁₁O₁₉.

In the method for forming a protective layer on a metallic turbine substrate according to the present invention, an aqueous solution is prepared, in which solution there can be easily dissolved a salt or an alkoxide having a cation which can act as a precursor, in other words which can form the ceramic oxide on the surface of the said metallic substrate.

A second component, comprising at least one substance selected from the group consisting of urea, hydrazine and its derivative, azine and its derivative is then dissolved in the aqueous solution.

The metallic substrate is then brought into contact with the solution and heated to a temperature in the range from 300°C to 800°C, preferably from 500°C to 700°C, until, after the solvent has been volatilized, a strongly exothermic reaction is initiated to form a thin layer of oxide on the surface of the metallic substrate.

Preferably, the first component is an inorganic salt comprising an anion selected from the group consisting of nitrate, nitrite, sulphate, halide, acetate, carboxylate, citrate, in other words salts soluble in aqueous solutions.

Preferably, the first component comprises a nitrate.

Even more preferably, the first component is selected from the group consisting of aluminium nitrate, manganese nitrate, lanthanum nitrate, yttrium nitrate, zirconium nitrate, cerium nitrate, barium nitrate, these components being capable of forming optimal ceramic oxides on metallic substrates for turbines.

Alternatively, it is also possible to use salts which can be decomposed by heat, such as titanium oxysulphate or alkoxides, for example tetraethylorthosilicate.

The second component is preferably urea.

A highly exothermic reaction takes place between the first component and the sacrificial fuel; if the reaction takes place between a nitrate and urea, it is of the following type:

x M(NO₃)_{y} + (3xy-y)/3 CO(NH₂)₂ → → MₓO_{y} + (3xy-y)/3 CO₂ + (9xy-2y)/6 N₂ + (6xy-2y)/3 H₂O

where M is the precursor of the oxide which is to be formed as the protective layer on the metallic substrate.

If the salts used as the first component are nitrates of Zr, La and Al, the reaction becomes:

ZrO(NO₃)₂ + 5/3 CO(NH₂)₂ → ZrO₂ + 5/3 CO₂ + 16/3 N₂ + 10/3 H₂O

La(NO₃)₃ + Mn(NO₃)₂ + 11 Al(NO₃)₃ + 95/3 CO(NH₂)₂ → → LaMnAl₁₁O₁₉ + 95/3 CO₂ + 152/3 N₂ + 190/3 H₂O

The reaction, which is thermally initiated, is self-sustaining because of the high exothermicity and is completed in a few tenths of a second with the formation of the solid ceramic product and the emission of gaseous species such as CO₂, H₂O and N₂. The sacrificial fuel can undergo partial thermal decomposition before the initiation of the main reaction with the formation of products which react with the salts by secondary reactions, which in all cases lead to the formation of the solid ceramic product and gaseous species such as CO₂, H₂O, N₂, and nitrogen oxides.

The solution can also comprise a third component acting as an adjuvant, for example ammonium nitrate, which reacts exothermically with the sacrificial fuel to increase both the temperature and the quantity of gas emitted.

Preferably, the adjuvant reaction takes place with urea, and in particular, if the adjuvant is ammonium nitrate, the following reaction takes place:

3 NH₄NO₃ + CO(NH₂)₂ → CO₂ + 4 N₂ + 8 H₂O

The presence of ammonium nitrate may require the use of additional quantities of fuel, not necessarily in a stoichiometric quantity, because any excess ammonium nitrate, as well as any excess fuel, is removed during synthesis by the decomposition and formation of gaseous products. The sacrificial fuel is therefore used in a stoichiometric quantity to react directly with the precursor salts or in a substoichiometric or superstoichiometric quantity, provided that it is sufficient to initiate and complete the process. The dimensions of the oxide particles forming the metallic layer and the corresponding degree of porosity will vary according to the proportions of salt to fuel and any adjuvant used.

The method for forming the protective layer according to the invention is preferably applied at atmospheric pressure and the reaction takes place at a temperature in the range from 300°C to 800°C, a range in which the initiation takes place and leads to the formation of the oxides which form the protective layer.

To achieve optimal results, the surface of the metallic substrate to be coated can be cleaned beforehand, by sandblasting for example, to promote the adhesion of the protective layer to the metallic substrate, and pre-heated before being brought into contact with the solution containing the reagents.

Advantageously, the step of bringing the solution into contact with the metallic substrate can be carried out by spraying with a spray gun, or by impregnation.

Generally, the sequence of steps of the method starts with the cleaning of the surface of the metallic component and then comprises a step of pre-heating the component in a furnace and the subsequent deposition of the reagent solution on the surface. After this, the substrate is kept in the furnace until the reaction is complete. The substrate is then taken out and blown with compressed air to remove any of the ceramic product which has not adhered sufficiently to the surface.

The protective layer which is obtained is generally very thin, with a thickness of approximately 5 µm for example, but the deposition of the protective layer can be repeated a number of times in an automatic way to produce final protective layers of the desired thickness, preferably in the range from 100 µm to 200 µm.

An examination of the characteristics of the method according to the present invention will clearly reveal the advantages which it provides.

In particular, this method can advantageously be used to deposit protective layers which may be either amorphous or crystalline, in which the particle sizes are of the order of microns or of the order of nanometres. Advantageously, the crystalline states are not subject to devitrification processes, with possible dimensional variations, when the component operates at high temperatures. The method can also be used for the deposition of protective layers generated by the successive deposition of a plurality of layers which may have different chemical compositions. Furthermore, the reaction conditions maintained during the process, the separation of the molecules of the reagents in the solution, the rapidity of the synthesis, and the evolution of considerable quantities of gas lead to the production of particles even down to nanometric sizes and enable the degree of porosity of the protective layer to be controlled.

Even more advantageously, the deposition method according to the present invention can be used to obtain a protective layer with a very fine and uniformly distributed porosity, which has excellent characteristics in respect of thermal insulation.

Advantageously, by varying the operating conditions of the illustrated method, for example by varying the temperature and the quantity of sacrificial fuel and ammonium nitrate, it is possible to obtain powders having a surface area varying in the range from 3 to 300 m²/g.

Advantageously, the deposition method according to the invention is also applicable to excessively large pores or to cavities which are formed accidentally in the first steps of production of the substrate.

Advantageously, the method according to the invention can also be used at temperatures which do not damage the structure of the metallic substrate.

Finally, the method according to the invention requires the use of very simple and economical equipment, such as a chamber furnace with resistors as the heating elements, and is therefore much more economical than known deposition methods. The method allows the introduction of further accessory thermal treatments, both in the intermediate steps of the deposition and at the end of this process. These treatments may have the purpose of crystallizing the deposited ceramic material, sintering the protective layer and improving the interface bond with the metallic substrate.

A crystallization treatment can be useful for stabilizing the structure of the surface layer, thus preventing the occurrence of structural and dimensional changes during service life. For example, LaMnAl₁₁O₁₉ deposited by the APS method is amorphous in nature and, if subsequently heated, shows the formation of large cavities and a decrease in mechanical strength because of the shrinkage caused by crystallization. The method which has been developed has the advantage of being able to eliminate the cavities due to crystallization and to consolidate the protective layer with further depositions.

The porosity of the layer can be decreased further by a final sintering treatment.

A final thermal treatment can improve the interface bond between the protective layer and the substrate by the activation of diffusion processes.

The temperatures to be used for crystallization, sintering and diffusion depend on the type of ceramic material forming the protective layer and can be specified from time to time, the only limitation being the maximum temperature which the substrate can withstand.

Finally, the method according to the invention can easily be automated; this is because the component can be moved continuously through a series of stations which carry out the successive steps of the method, namely the pre-heating step, the spraying of the solution, the reaction and the blowing. Lastly, the series of stations can be joined up to form a cycle.

Further characteristics of the present invention will be made clear by the following description of an example, provided solely for illustrative purposes and without restrictive intent, of a method for depositing a protective layer of lanthanum hexaluminate.

The first step is to form a solution containing:
- 7.36 g of aluminium nitrate;
- 0.33 g of manganese nitrate;
- 0.54 g of lanthanum nitrate;
- 3.24 g of urea, and
- 5 ml of water.

The solution produced in this way is sprayed, until complete wetting is achieved, on to a metallic substrate pre-heated in a furnace programmed to a constant temperature of 600°C. The metallic substrate treated in this way is placed back in the furnace at 600°C for two minutes. The metallic substrate is then taken out of the furnace and blown with compressed air so as to remove the excess material, in other words that which has not adhered to the said metallic substrate. The procedure is repeated 20 times to produce a protective layer with a thickness of 100 µm.

## Claims

1. Method for forming a protective layer on a metallic turbine substrate, **characterized in that** it comprises the steps of:
- preparing an aqueous solution comprising a first component comprising at least a salt or an alkoxide, at least partially soluble in water, having at least a cation which can act as a precursor of a ceramic oxide;
- dissolving in the said aqueous solution a second component comprising at least one substance selected from the group consisting of urea, hydrazine and its derivatives, azine and its derivatives-, acting as sacrificial fuel;
- bringing the metallic substrate into contact with the solution;
- heating the metallic substrate to a temperature in the range from 300°C to 800°C until, after the solvent has been volatilized, a strongly exothermic reaction is thermally initiated and leads to the formation of oxides which form a protective layer on the surface of the said metallic substrate;
and by the fact that the reaction to form an oxide is self-sustaining.

2. Method according to Claim 1, **characterized in that** the said second component is urea

3. Method according to any Claims 1 or 2, **characterized in that** the said aqueous solution comprises ammonium nitrate as the third component.

4. Method according to any one of the preceding claims, **characterized in that** the said first component is a salt having an anion selected from the group consisting of nitrate, nitrite, sulphate, halide, acetate, carboxylate and citrate.

5. Method according to Claim 4, **characterized in that** the said first component is a salt having a nitrate as its anion.

6. Method according to Claim 5, **characterized in that** the said nitrate salt comprises an element selected from the group consisting of aluminium, manganese, lanthanum, zirconium, cerium, barium and yttrium.

7. Metallic turbine substrate, comprising a porous protective layer **characterized in that** the said protective layer is an oxide of a ceramic nature produced according to any one of the preceding claims.

8. Metallic substrate according to Claim 7, **characterized in that** the said protective layer comprises an oxide selected from the group consisting of ZrO₂, ZrO₂+Y₂O₃, ZrO₂+CaO, Al₂O₃, Al₂O₃+SiO₂, Al₂O₃+TiO₂, CeO₂, BaZzO₃, Y₃Al₅O₁₂, LaMgAl₁₁O₁₉, LaMnAl₁₁O₁₉.

9. Metallic substrate according to Claim 8, **characterized in that** the said protective layer is based on LaMnAl₁₁O₁₉.

## Patentansprüche

1. Verfahren zum Ausbilden einer Schutzschicht auf einem Metallsubstrat einer Turbine, **dadurch gekennzeichnet, dass** dieses die Schritte umfasst:
- Präparieren einer wässrigen Lösung mit einer ersten Komponente umfassend wenigstens ein Salz oder ein Alkoxid, das wenigstens teilweise in Wasser löslich ist, mit wenigstens einem Kation, welches als ein Vorläufer eines Keramikoxids wirken kann;
- Lösen einer zweiten Komponente in dieser wässrigen Lösung, umfassend wenigstens eine Substanz, ausgewählt aus der Gruppe bestehend aus Harnstoff, Hydrazin und seine Derivate, Azine und seine Derivate, die als Opferbrennmittel wirken;
- Bringen des Metallsubstrats in Kontakt mit der Lösung;
- Erwärmen des Metallsubstrats auf eine Temperatur im Bereich von 300°C bis 800°C, bis, nachdem das Lösemittel verflüchtigt wurde, eine stark exotherme Reaktion thermisch initiiert wird und zu der Bildung von Oxiden führt, welche eine Schutzschicht auf der Oberfläche des Metallsubstrats bilden;
und durch die Tatsache, dass die Reaktion, ein Oxid zu bilden, selbsterhaltend ist.

2. Verfahren nach Anspruch 1, **dadurch gekennzeichnet, dass** die zweite Komponente Harnstoff ist.

3. Verfahren nach einem der Ansprüche 1 oder 2, **dadurch gekennzeichnet, dass** die wässrige Lösung Ammoniumnitrat als die dritte Komponente umfasst.

4. Verfahren nach einem der vorhergehenden Ansprüche, **dadurch gekennzeichnet, dass** die erste Komponente ein Salz mit einem Anion ist, ausgewählt aus der Gruppe bestehend aus Nitrat, Nitrit, Sulfat, Halogenid, Acetat, Carboxylat und Citrat.

5. Verfahren nach Anspruch 4, **dadurch gekennzeichnet, dass** die erste Komponente ein Salz mit Nitrat als ein Anion ist.

6. Verfahren nach Anspruch 5, **dadurch gekennzeichnet, dass** das Nitratsalz ein Element umfasst, ausgewählt aus der Gruppe bestehend aus Aluminium, Mangan, Lanthan, Zirkonium, Cer, Barium und Yttrium.

7. Turbinen-Metallsubstrat, mit einer porösen Schutzschicht, **dadurch gekennzeichnet, dass** die Schutzschicht ein Oxid aus einer keramischen Natur ist, hergestellt nach einem der vorhergehenden Ansprüche.

8. Metallsubstrat nach Anspruch 7, **dadurch gekennzeichnet, dass** die Schutzschicht ein Oxid umfasst, ausgewählt aus der Gruppe bestehend aus ZrO₂, ZrO₂+Y₂O₃, ZrO₂+CaO, Al₂O₃, Al₂O₃+SiO₂, Al₂O₃+TiO₂, CeO₂, BaZrO₃, Y₃Al₅O₁₂, LaMgAl₁₁O₁₉, LaMnal₁₁O₁₉.

9. Metallsubstrat nach Anspruch 8, **dadurch gekennzeichnet, dass** die Schutzschicht auf LaMnAl₁₁O₁₉ basiert.

## Revendications

1. Procédé de formation d'une couche protectrice sur un substrat de turbine métallique, **caractérisé en ce qu'**il comprend les étapes suivantes :
- préparation d'une solution aqueuse comprenant un premier composant comprenant au moins un sel ou un alcoxyde, au moins partiellement soluble dans l'eau, ayant au moins un cation qui peut jouer le rôle de précurseur d'un oxyde céramique ;
- dissolution dans ladite solution aqueuse d'un second composant comprenant au moins une substance choisie dans le groupe constitué de l'urée, de l'hydrazine et de ses dérivés, de l'azine et de ses dérivés, jouant le rôle de combustible sacrificiel ;
- mise en contact du substrat métallique avec la solution ;
- chauffage du substrat métallique à une température dans la plage de 300°C à 800°C jusqu'à ce que, après volatilisation du solvant, une réaction fortement exothermique soit thermiquement initiée et conduise à la formation d'oxydes qui forment une couche protectrice sur la surface dudit substrat métallique ;
et par le fait que la réaction de formation d'un oxyde soit auto-entretenue.

2. Procédé selon la revendication 1, **caractérisé en ce que** ledit second composant est l'urée.

3. Procédé selon l'une quelconque des revendications 1 ou 2, **caractérisé en ce que** ladite solution aqueuse comprend du nitrate d'ammonium comme troisième composant.

4. Procédé selon l'une quelconque des revendications précédentes, **caractérisé en ce que** ledit premier composant est un sel ayant un anion choisi dans le groupe constitué d'un nitrate, d'un nitrite, d'un sulfate, d'un halogénure, d'un acétate, d'un carboxylate et d'un citrate.

5. Procédé selon la revendication 4, **caractérisé en ce que** ledit premier composant est un sel comprenant un nitrate comme son anion.

6. Procédé selon la revendication 5, **caractérisé en ce que** ledit sel de nitrate comprend un élément choisi dans le groupe constitué de l'aluminium, du manganèse, du lanthane, du zirconium, du cérium, du baryum et de l'yttrium.

7. Substrat de turbine métallique, comprenant une couche protectrice poreuse, **caractérisé en ce que** ladite couche protectrice est un oxyde de nature céramique produit selon l'une quelconque des revendications précédentes.

8. Substrat métallique selon la revendication 7, **caractérisé en ce que** ladite couche protectrice comprend un oxyde choisi dans le groupe constitué de ZrO₂, ZrO₂+Y₂O₃, ZrO₂+CaO, Al₂O₃, Al₂O₃+SiO₂, Al₂O₃+TiO₂, CeO₂, BaZrO₃, Y₃Al₅O₁₂, LaMgAl₁₁O₁₉ et LaMnAl₁₁O₁₉.

9. Substrat métallique selon la revendication 8, **caractérisé en ce que** ladite couche protectrice est à base de LaMnAl₁₁O₁₉.
